

Jan. 9, 1940.

P. H. DOWLING

2,186,781

ELECTRICAL RECTIFIER

Filed March 19, 1938



Fig. 1.



Fig. 2.



Fig. 3.



Fig. 4.

INVENTOR  
Philip H. Dowling.  
BY *A. L. Venelle*  
HIS ATTORNEY

## UNITED STATES PATENT OFFICE

2,186,781

## ELECTRICAL RECTIFIER

Philip H. Dowling, Forest Hills, Pa., assignor to  
 The Union Switch & Signal Company, Swiss-  
 vale, Pa., a corporation of Pennsylvania

Application March 19, 1938, Serial No. 196,912

3 Claims. (Cl. 175—366)

My invention relates to electrical rectifiers, and particularly to electrical rectifiers of the copper oxide type.

One object of my invention is to improve the rectifying characteristics of rectifiers of the type described.

A feature of my invention comprises manufacturing copper oxide rectifiers from copper containing a small amount of another metal, such, for example, as lead.

I shall describe one form of rectifiers embodying my invention, and shall then point out the novel features thereof in claims.

In the accompanying drawing, Fig. 1 is a view showing in side elevation one form of copper blank ready to be manufactured into a rectifier element in accordance with my invention. Fig. 2 is a view showing a number of blanks assembled on a support as they appear during one step in the process of manufacture. Fig. 3 is a vertical sectional view showing, in an exaggerated form, a rectifier element as it appears in another step in the process of manufacture. Fig. 4 is a view showing a completed rectifier element constructed in accordance with my invention.

Similar reference characters refer to similar parts in all four views.

In the process of manufacturing copper oxide rectifiers, as it is now generally practiced, a number of copper blanks, which may, for example, be similar to the blank A shown in Fig. 1, are first cleaned in any suitable manner as by an acid etch, and these blanks are then assembled in pairs on a suitable support B in the manner shown in Fig. 2 so that the blanks of each pair have their adjacent faces A<sup>1</sup> in contact. The blanks are then heated in the presence of air in an electric furnace, the temperature of which is usually maintained at about 1860° F. This heating of the blanks causes a layer of red or cuprous oxide to be formed on the blanks, and is continued until the cuprous oxide layer is of the desired thickness. After a sufficient amount of oxide has been formed on the copper blanks, these blanks are then transferred immediately to a second furnace which is maintained at a temperature of approximately 1050° F., and are allowed to remain in this latter furnace only for a sufficient length of time to permit them to cool down to the temperature of the second furnace. The oxidized blanks are then removed from the second furnace and are suddenly cooled or "quenched" as by plunging the blanks into cold water or a current of cold air. Each blank then appears as shown in Fig.

3 from which it will be seen that each blank A is now covered with an inner coating D of cuprous or red oxide of copper and a thin outer coating C of black oxide of copper. It will also be seen from an inspection of Fig. 3 that the flat face A<sup>2</sup> of the blank which is exposed during the oxidizing process, that is to say, the lower face, has a much heavier oxide coating than the upper face. Each blank is next treated to remove the black oxide from the lower face of the blank, and both the black and red oxide from the upper face, after which the blank will appear as shown in Fig. 4. One process which is particularly suitable for removing the excess oxide from the blanks is described and claimed in Letters Patent of the United States No. 2,094,642 granted to me on October 5, 1937. As a last step, the electrical contact to the exposed face of the cuprous oxide remaining on the blank is improved, as by rubbing into the face powdered petroleum coke.

Rectifier elements of the type described exhibit the characteristic of offering a relatively low resistance to current flowing through the element from the cuprous oxide to the copper and a relatively high resistance to the flow of current through the element in the opposite direction. The resistance of the element in the low resistance direction will hereinafter be referred to as the conducting resistance, while the resistance of the element in the high resistance direction will hereinafter be referred to as the blocking resistance.

Rectifier elements of the type described also exhibit the characteristic that when a voltage is applied to them in the high resistance or blocking direction, the high or blocking resistance will decrease at first relatively rapidly and then somewhat more slowly with time until it obtains an apparently stable value which may be considerably less than the initial value. The stable virtual value of the reverse current when an alternating voltage is applied to the rectifier is increased due to this effect, and this effect accordingly in some instances determines the voltage for which the rectifier is capable of effecting satisfactory rectification in service. This change in blocking resistance with time is ordinarily known as "creep", or "reverse creep", and is usually temporary in character, the apparent resistance in the reverse direction gradually returning toward its original value when the voltage is removed.

I have found that when rectifier elements are manufactured by the process previously de-

scribed, the presence in the copper from which the elements are manufactured of certain metallic impurities appears to materially affect the characteristics of the rectifier elements. One such impurity which I have found to be particularly effective in affecting the characteristics of the elements is lead, the presence of which in proper amounts increases the reverse resistance, decreases the tendency to creep, and also decreases the aging of the rectifiers in the blocking direction. The lead to be effective should be present in a concentration of at least .001% by weight, and a concentration of .005% by weight gives particularly good results. In certain applications where exceptional reverse current stability is of more importance than a low resistance in the conducting direction, concentrations above .005% by weight may at times be found to be useful. In no event, however, should the concentration of the lead be large enough to interfere with the smelting and rolling process by which the sheets or strips from which the blanks are punched are formed, nor should it be so large as to interfere with the adherence of the oxide layer to the mother metal.

One advantage of the use of a copper body containing lead for the manufacture of rectifier elements is that it reduces the detrimental effects on the blocking resistance of the presence of anodic impurities during the manufacturing process.

Although I have herein shown and described only one form of electrical rectifiers embodying my invention, it is understood that various changes and modifications may be made therein within the scope of the appended claims without departing from the spirit and scope of my invention.

Having thus described my invention, what I claim is:

1. A copper oxide rectifier formed from a copper body containing approximately .001% by weight lead.

2. A copper oxide rectifier formed from a copper body containing approximately .005% by weight lead.

3. A copper oxide rectifier formed from a copper body containing between .001% and .005% by weight lead.

PHILIP H. DOWLING.